

1,115,042.

A. B. WARING.

FELT HAT.

APPLICATION FILED NOV. 19, 1912.

Patented Oct. 27, 1914.

*Fig. 1,*



*Fig. 2,*



WITNESSES  
P. J. Garboe  
F. Graves.

INVENTOR  
Arthur B. Waring  
BY  
E. W. Marshall  
ATTORNEY

# UNITED STATES PATENT OFFICE.

ARTHUR B. WARING, OF NEW YORK, N. Y.

## FELT HAT.

1,115,042.

Specification of Letters Patent.

Patented Oct. 27, 1914.

Application filed November 19, 1912. Serial No. 732,203.

*To all whom it may concern:*

Be it known that I, ARTHUR B. WARING, a citizen of the United States of America, and a resident of New York, county and 5 State of New York, have invented certain new and useful Improvements in Felt Hats, of which the following is a specification, reference being had to the accompanying drawings, forming a part thereof.

10 My invention relates to felt hats, and its object is to provide a hat of novel and attractive appearance. In general this novel effect is attained by making the different portions or surfaces of a hat of different 15 colors or character.

I will now describe my invention in the following specification and then point out the novel features thereof in appended claims.

20 Both of the two figures of the drawings are perspective views of hats embodying my invention and similar characters of reference are used in both of the figures to designate corresponding parts.

25 The hat illustrated in the drawings is a soft felt hat of which 10 is the crown, 11 the upper surface of the brim, and 12 the under surface of the brim.

In order that this invention may be fully 30 understood I will describe one way in which the hat may be made. A mixture is made of felting material and a small proportion of non-felting material such for example, as animal fibers and vegetable fibers. As a 35 more specific example the mixture may be of 85% fur and 15% ramie. A hat body of this mixture is formed and then shrunk. In the shrinking process the fur felts and covers the ramie so that the latter does not

40 show upon the surface. The hat body thus formed may be pounced or abraded a sufficient amount to bring it to a smooth surface without materially altering its looks or appearance. A further amount of pouncing, 45 especially if a rougher abrasive such as coarser sand-paper is used, will rub off enough of the exterior felted fur fibers to disclose the unfelted intermingled ramie fibers which were beneath the surface. The 50 faces thus treated will have a different appearance in color or in character from the parts which are not thus subjected to further abrasion. This is because the two kinds of fiber are unlike in looks. In fact the

contrast between them may be heightened 55 by artificially coloring one or the other of the materials. The ramie may be left white or dyed any desired color. If it is dyed it is preferable to color it before it is mixed with the fur. If the fur is dyed it is better 60 to do this after the shrinking process because dyeing decreases its felting properties. This may be done by dyes which have little or no effect upon the ramie. The process of making such a hat body is more fully 65 described in a co-pending application for patent Serial No. 732,202, filed by me herewith.

It is my intention to subject some of the surfaces of such a hat to more abrasion than others to thereby obtain a contrast in appearance between the different surfaces. Let us assume that the fur is dyed black but the ramie is allowed to retain its original whiteness. If the crown and the under surface of the brim of such a hat have 75 the outside felted fibers rubbed off until the unfelted fibers appear, they will assume a gray color, as is represented at 10 and 12 in Figure 1, while the upper surface 11 of the rim retains its black color. Or if preferred the 80 crown and under surface of the brim may be left black as at 10<sup>A</sup> and 12<sup>A</sup> in Fig. 2, and the upper surface 11<sup>A</sup> of the brim made gray. Of course with a gray crown the upper surface of the brim may be gray and 85 its under surface black, or both surfaces of the brim black, or with a black crown the upper surface of the brim may be black and its under surface gray or both surfaces of the brim gray. Or with different degrees of 90 abrasion different shades of gray may be obtained. In this manner novel and attractive effects are produced.

The foregoing is given as an example of the way hats may be made according to this 95 invention. I do not limit myself to the use of fur and ramie, as wool and some other non-felting material such as silk may be used. Nor do I limit myself to the specific proportions of the elements cited 100 merely as an example. Any desired combinations of colors may be used and if desired the non-felting fibers may be darker than the others instead of lighter. They may even be of the same color but of different 105 character so long as the rubbed off surface or surfaces contrast in appearance from those which are not rubbed off. It is also

possible to obtain somewhat similar results by rubbing off one or more of the outer surfaces of a surface-dyed fabric.

What I claim is:

- 5 1. A felt hat made of a fabric having non-felting fibers intermingled with the felting fibers under the surface thereof with the felting fiber surface removed from one or more broad hat surfaces to disclose the 10 non-felting fibers and to contrast with other surfaces of the hat.
- 15 2. A felt hat made of a fabric having non-felting fibers unlike in appearance but mingled with the felting fibers beneath the surface thereof with the felting fiber surface removed from one or more broad hat surfaces to disclose the non-felting fibers and to contrast with other surfaces of the hat.
- 20 3. A felt hat made of a fabric having vegetable fibers intermingled with animal fibers beneath the surface thereof with the

animal fiber surface removed from one or more broad hat surfaces to disclose the vegetable fibers and to contrast with other surfaces of the hat, said animal and vegetable 25 fibers being unlike in appearance.

4. A felt hat having a crown surface, an upper rim surface, and an under rim surface, and made of a fabric having non-felting fibers intermingled with animal fibers 30 beneath the surfaces of the fabric, said animal fibers and non-felting fibers being of unlike colors, with the animal fiber surface of the fabric removed from one or more broad hat surfaces to contrast with other 35 surfaces or surface of the hat.

In witness whereof, I have hereunto set my hand this 16th day of November 1912.

ARTHUR B. WARING.

Witnesses:

ERNEST W. MARSHALL,  
JULIUS TACKMAN.

Copies of this patent may be obtained for five cents each, by addressing the "Commissioner of Patents, Washington, D. C."